

# UNITED STATES PATENT OFFICE.

HENRY DREYFUS, OF BASEL, SWITZERLAND.

## UNINFLAMMABLE CELLULOID SUBSTITUTE AND METHOD OF MAKING THE SAME.

1,181,858.

Specification of Letters Patent.

Patented May 2, 1916.

No Drawing. Application filed October 2, 1911, Serial No. 652,444. Renewed December 11, 1915. Serial No. 66,397.

*To all whom it may concern:*

Be it known that I, HENRY DREYFUS, doctor of philosophy, chemist, a citizen of the Republic of Switzerland, residing at 5 Basel, Switzerland, (whose post-office address is 69 Schützenmatzstrasse, Basel, Switzerland,) have invented an Uninflammable Celluloid Substitute and Method of Making the Same, of which the following 10 description is a specification.

The production of a non-inflammable celluloid has been the subject of much research during late years, and either with nitro-cellulose in combination with camphor or 15 camphor substitutes capable of reducing inflammability, or with acetyl cellulose and camphor or camphor substitutes. Although many such substitutes have been proposed, 20 none of them has been capable of replacing camphor, as in general they have not fulfilled the requirements demanded of a camphor substitute. It has to be borne in mind that for such a substitute in the celluloid manufacture, not only its qualitative character has to be examined, but the relative 25 proportions also play a great part, for any other substitute requires graduation in the quantities to be employed, just as camphor does, and the value of a substitute can only be 30 judged from the finished celluloid, from which it can be seen whether the resulting material is brittle directly, or only becomes brittle after some time, or is too soft or possesses any other defects. The specification 35 of German Patent No. 145,106 describes *inter alia* a process for the production of celluloid-like substances in which phenol is used as a solvent. Nevertheless only elastic or horn-like products are obtained according 40 to that process; moreover the process is hardly capable of practical employment owing to the disagreeable odor, and moreover the production of a celluloid substitute would be impossible according to the working 45 indicated in the patent specification.

In specification of German Patent 188,542 a process for the production of celluloid-like substances is described, using tetrachlorethane. The production of a real celluloid substitute however, requires that the 50 same shall be capable of being worked upon the same machines as those employed for ordinary celluloid, and in particular calenders or rollers and presses. Especially

the rollers are necessary in order to produce 55 various designs or patterns, such as tortoise-shell, etc. If one worked according to this patent specification, using acetyl celluloses obtained according to the German patent specifications therein mentioned, *e. g.*, 60 163,316; 159,524, etc., one would not obtain a celluloid substitute. One reason for this is that the said acetyl celluloses are difficultly soluble, but even an excess of solvent would not overcome the difficulty, as one 65 would then only obtain sticky masses incapable of being worked on the machines, and which on prolonged drying on calender rollers and evaporation of the solvent would return to this original condition. How important is the part played by the degree of 70 solubility of the acetyl cellulose employed, is shown by the fact that there is also known a process wherein (owing to the too small solubility of the cellulose esters) these acetates are to be replaced by so-called sulfoacetates and phosphoacetates, the solvent 75 capacity of which for the phosphoric esters of phenols, naphthols, cresols, acetins and others is said to be considerably greater and 80 the formation of celluloid to be therefore possible. Moreover in the specification of 85 German Patent 188,542 the mass is taken direct to presses for the formation of objects or blocks, etc. But the rollers are essential 90 for the production of designs, and moreover they allow of further working up, and inspection of the mass. It is altogether impossible however, to work up on rollers the masses obtained from acetyl cellulose 95 according to the said patent specification, as the same would simply break and crumble as the solvent evaporates, instead of blending under the calendering action into homogeneous coherent plastic masses, becoming 100 transparent, which will form viscous sheets or foils and can easily be cut with a knife. The production of designs or patterns by the introduction of dissolved or undissolved coloring matters or fillers, is entirely impossible, and apart from this fact the material is brittle, more or less opaque and 105 spotted with white. These are all products soluble it is true, in tetrachlorethane, but which are nevertheless precipitated from their solutions therein, upon the addition of alcohol; even the product of German Patent 159,524 which is more easily soluble in

tetrachlorethane will bear only a very little alcohol and cannot be used for the production of celluloid, especially on account of its too small solubility. Further it has also been incorrectly assumed that the rapidity of evaporation of the solvents used, as for instance acetone, is the cause of the substance being brittle, owing to the material drying too quickly. It has been found in the present process that the brittleness is due *inter alia* to the character of the acetyl celluloses employed, and in particular, to their capacity for dissolving in tetrachlorethane being much too small; even if an excess of tetrachloroethane is used for solution, this excess is evaporated again in the working up of the product and the mass again becomes opaque and crumbly and brittle, so that it is impossible to work it on rollers. Moreover it is not possible in accordance with the aforesaid assumption to obtain a useful product, and this apart from the fact that the camphor added allows the inflammability to persist. Besides the important part played by the quality of the acetyl celluloses employed, importance also attaches to the relative proportions of tetrachlorethane and alcohol or its substitutes; for if too much alcohol is used, it acts as a precipitant and the formation of celluloid is impossible, whereas with little alcohol the quantity of tetrachlorethane employed must be preferably increased.

I have found a process which allows of the employment of tetrachlorethane for the production of a real celluloid substitute, having all the desirable properties of ordinary celluloid. The process enables the cellulose acetates or cellulose esters to be worked on the same machines as ordinary celluloid and allows of producing designs, patterns or colorings in the usual manner for example with dyestuffs soluble in alcohol or diluted alcohol, or with filling materials such as asbestos in powder, or mineral substances such as bronze, zinc white, barium compounds, etc. The new process depends on the quality of the cellulose acetates employed and to some extent on the quantity of the substance to be used, such as tetrachlorethane and alcohol or the substitutes of the latter, both among themselves and relatively to the particular acetyl celluloses or other cellulose esters used. It has been found in particular that for the manufacture of a real celluloid substitute, those cellulose esters which are described and claimed in my applications 652,442 filed concurrently herewith and 782,530, filed August 1, 1913, which in mixtures of alcohol-tetrachlorethane give highly concentrated solutions, are especially suitable. Some of them are capable of giving solutions of up to 50 per cent. and more of acetyl cellulose in a mixture of about equal vol-

umes of tetrachlorethane and alcohol, especially on warming. The behavior of these solutions for example when worked up in presses is such that when heated for example at 70 to 90° C., they become thickly or 70 slightly fluid, and transparent, while on cooling they solidify again into more or less soft to hard transparent masses, which can be worked up in an analogous manner to ordinary celluloid; and these solutions 75 possess the advantages over ordinary celluloid that they can be cast and molded direct into objects of all kinds. The total quantity of the solvents employed, as tetrachlorethane and alcohol or its substitutes, 80 should not on the average exceed together more than about 80 to 100 per cent. of the cellulose ester used. According as it is desired to make a harder or a softer celluloid substitute, the proportions can be reduced 85 or increased and oils, such as castor oil or the like may be added if desired. The production of celluloid from cellulose esters characterized by their solubility is however not in every case dependent upon the employment of alcohol or the substitutes of the latter, as it has been found that these cellulose esters can also be used without alcohol although it is true with certain disadvantages. In this case, however, it has 90 been found that to provide for the working of the mass, it is preferable to use about 100 to 150 per cent. of tetrachlorethane, relatively to the weight of acetyl cellulose instead of for example only 50 per cent., in 100 order to effect the melting and uniting of the mass and to enable the same to be worked upon rollers. If too much tetrachlorethane is used, however, the mass cannot be worked up and among other things 105 it is hardly possible to produce designs or patterns on calender rollers with organic or mineral coloring matters, or to introduce filling substances as required. Even by evaporation it is very difficult to remove the 110 excess of solvent, and the quality of the resulting celluloid is detrimentally affected and the latter rendered useless for many purposes. The success of the present process depends upon the employment of acetyl 115 celluloses or cellulose esters referred to possessing the above described properties and also upon the proportions of the added substances among themselves and also together in relation to the weight of the cellulose 120 esters employed. It has further been found that the chlorin derivatives of ethylene and ethane allied to tetrachlorethane *e. g.* penta-chlorethane, dichlorethylene, and trichlorethylene, although chemically they are 125 very closely related to each other and to tetrachlorethane and although they could hardly be expected to show a different behavior relatively to cellulose esters, do nevertheless show individually and in mix- 130

tures of some or all of them a great difference in their behavior toward acetyl celluloses. Pentachlorethane has already been used with the employment of a solvent such as chloroform, in which the acetyl cellulose is first dissolved, in order to produce films therefrom. The subject of the present invention, however, represents *inter alia* the very employment of the cellulose acetates which are capable of giving highly concentrated solutions in alcohol and tetrachlorethane, for as has been found in the present process, even when pentachlorethane is employed, the hitherto known acetyl celluloses which are soluble in chloroform cannot be used for the production of celluloid, as their capacity for dissolving in this solvent is far too small.

The British specification, 14,364 of 1910 describes a method in which pentachlorethane is used with addition of solvents for acetyl celluloses, such as chloroform and acetone, for the manufacture of films, threads and sheets. But according to the aforesaid process it is only possible to obtain solutions for celluloid, and the proportions employed are so great that working on the machines usual for celluloid is not possible; only sticky and liquid masses would be obtained. A real substitute that can be worked on the same machines is impossible with said process, as is also the coloring with organic and mineral coloring matters, and the largely excessive quantities of solvents used are employed in a useless way. Moreover in said process all cellulose acetates are employed. Just as with tetrachlorethane it has also been found that only the acetyl celluloses giving concentrated solutions in alcohol-tetrachlorethane can be employed, and on the other hand the proportions of the solvents employed (alcohol and pentachlorethane), both in relation to each other and in relation to the acetyl celluloses, are of particular importance, for if for example too much alcohol is added relatively to the pentachlorethane, it acts as a precipitating agent so that the formation of celluloid is impossible. It has further been found that for the production of a good celluloid substitute, it is of advantage to employ on an average 80 to 100 per cent. of a mixture of pentachlorethane and alcohol or its substitutes, relatively to the weight of the cellulose acetate employed but these limits may be departed from to a certain extent according as a harder or softer celluloid is required.

In using pentachlorethane it has been found preferable to work with a mixture of equal volumes of pentachlorethane and alcohol; it is thus possible and particularly by heating, to produce solutions containing up to 50 per cent. and more of cellulose acetates and which can be worked up on the ordinary

celluloid machines. A two-fold technical advantage is thus obtained; on the one hand the possibility of producing a useful celluloid substitute by limiting the total quantities of alcohol and pentachlorethane employed, and on the other hand the restricted quantity of solvents considerably reduces the cost price of the celluloid. It has further been found that, while tetrachlorethane which of itself and without addition of alcohol or substitutes thereof, is capable of forming a celluloid substitute with the acetyl celluloses very soluble in mixtures of tetrachlorethane and alcohol, pentachlorethane is incapable of itself of forming plastic masses with these acetyl celluloses. If for example the acetocelluloses are treated with pentachlorethane in the same manner as with tetrachlorethane, the acetyl cellulose remains indifferent, even when heated and stirred. The surprising fact has been discovered, however, that if tetrachlorethane is added to pentachlorethane, for example in equal volumes, or more or less of the one or the other according to circumstances, the pentachlorethane is capable of forming a celluloid substitute even although less advantageously without addition of alcohol or its substitutes. The same result is obtained by employing pentachlorethane mixed with methyl acetanilid or other camphor substitutes. Moreover it has been found that trichlorethylene, which of itself has no dissolving capacity for the particular acetyl celluloses, nevertheless in admixture with pentachlorethane and with tetrachlorethane is capable of forming celluloid masses with acetyl cellulose, and especially in combination with alcohol or its substitutes. This latter fact is in contradiction with the British Patent 16,932 of 1910 and French Patent 418,309 which state that trichlorethylene neither alone nor in combination with alcohol has any dissolving capacity for acetates of cellulose, for it has been found in the present invention that the cellulose acetates referred to which give concentrated solutions in alcohol-tetrachlorethane give concentrated solutions in a hot mixture of trichlorethylene and alcohol (for example in a mixture of equal parts by volume of trichlorethylene and alcohol) which solutions set on cooling. It has also been found that dichlorethylene in combination with other chlorin derivatives of acetylene, such as penta- and tetra-chlorethane, with or without alcohol show an analogous behavior with cellulose acetates; the only difference is, as already known, that dichlorethylene of itself has a certain dissolving capacity for certain cellulose acetates. It has also been found that the results obtained according to the present invention are also quite different from those of the process of French Patents 412,797 and 419,530, and English Patents 1441 of 1910 and 12,979 of 1909 which state,

that it had only previously been possible to produce thin coatings with acetyl cellulose and that the production of celluloid is only possible by employing alcohol-benzol. In 5 the present invention it has been found that the result depends only on the quality or character of the cellulose acetates or cellulose esters employed and the qualitative and quantitative selection of the solvents and so-called additions *inter se*, and in relation to the cellulose esters employed. I have found that only agents should be employed which of themselves, or in combination with liquids or other substances, preferably possess 10 the greatest dissolving capacity for the acetyl celluloses referred to, and that precipitating agents, or agents which lower the solvent powers are to be avoided. That the aforesaid processes (the French and English 15 patents above referred to) are incorrect is shown by the following: If for example benzene is taken as the volatile agent or alone as the solvent, and one adds the there employed camphor substitutes, the acetyl cellulose remains almost indifferent even on heating, as the benzene in combination with the camphor substitutes, acts as a precipitating agent, or as a solubility reducing agent. If 20 on the other hand one takes for example a mixture of equal parts of alcohol and benzene, or petroleum spirit instead of benzene, this mixture even with additions of camphor substitutes, acts as a precipitating agent. The acetyl cellulose remains indifferent, and 25 on the other hand become so soaked with this precipitating agent combined with the added camphor substitute, that the removal of the mixture is extremely difficult. The result is the same when other volatile liquids are employed, as for instance carbon disulfid, etc. In the present process therefore, the additions of the volatile liquids in 30 these aforesaid processes and the special preparatory treatments of the cellulose acetates connected with the same are not necessary; consequently the new process presents a technical advantage as compared therewith apart 35 from the further advantages of the present invention.

50 The present process is illustrated by the following examples:

Example 1: 80 kilos of cellulose acetate, easily soluble in alcohol-tetrachlorethane, are mixed with about 40 liters of alcohol and 40 55 kilos of tetrachlorethane and kneaded to a sufficient extent in a malaxator, preferably while warm; the mass becomes homogeneous and clear. It is then worked up on rollers and in presses, and the resulting block is cut 60 for example into plates or sheets of the desired thickness, which can further be dried and dressed or polished according to requirements. To the above mixture there may be added at the beginning, or later, such sub-

stances as castor oil, or mineral or organic 65 coloring matters, or filling substances according to the use in view. If for example it is intended to produce an imitation tortoise shell the mass is divided into two or more equal or unequal parts during the 70 working up on rollers operation. Taking equal parts for example, one of the parts may be colored with organic coloring matters, for example Bismarck brown, or combined with blue or other coloring matters, 75 such as methylene blue, Victoria blue, etc., according to the effect desired, and after the coloring it is mixed with the other uncolored part by suitable working upon rollers. In this example 5 kilos of methyl acetyl 80 acetanilid, or other suitable camphor substitute may be added. The 40 kilos of tetrachlorethane may be replaced by 40 kilos of a mixture of equal parts of tetra- and penta-chlorethane.

Example 2: 20 kilos of cellulose acetate, 85 easily soluble in alcohol-tetrachlorethane are mixed with 20 liters of alcohol and 32 kilos of tetrachlorethane and further worked up as in the preceding example. The material is distinguished by particular 90 softness.

In these examples the proportions of the substances used may be varied somewhat, both relatively to each other and to the cellulose acetate referred to and the constituents of the dissolving mixtures can likewise be varied. The masses obtained in these examples instead of being further worked up on the usual celluloid machines, may be cast in molds directly or after addition of filling materials, oils, and so forth and films or other objects of all kinds may be made from them. 100

The term "alcohol" as used in the appended claims is intended to cover the use 105 of alcohol substitutes.

What I claim is:—

1. In a process of making a celluloid substitute, the step which comprises dissolving, in a mixture comprising alcohol and a 110 chlorinated hydrocarbon, a cellulose ester which is readily soluble therein, in proportions to form a solution containing not less than 29% of said ester.

2. In a process of making a celluloid substitute, the step which comprises dissolving, in a mixture comprising alcohol and a chlorinated hydrocarbon, a cellulose acetate which is readily soluble therein, in proportions to form a solution containing not less than 120 115 29% of said acetate.

3. In a process of making a celluloid substitute, the step which comprises dissolving, in a mixture comprising alcohol and tetrachlorethane, a cellulose ester which is 125 readily soluble therein, in proportions to form a solution containing not less than 29% of said ester.

4. In a process of making a celluloid substitute, the step which comprises dissolving, in a mixture comprising alcohol and a chlorinated hydrocarbon, a cellulose ester which is readily soluble therein, in proportions to form a solution containing about 50% of said ester.
5. In a process of making a celluloid substitute, the step which comprises dissolving, 10 in a mixture comprising alcohol and a chlorinated hydrocarbon, a cellulose ester which is readily soluble therein, in proportions to form a solution containing not less than 29% of said ester, together with a suitable proportion of an oil.
6. In the manufacture of a celluloid substitute, the process which comprises dissolving, in a mixture comprising alcohol and a chlorinated hydrocarbon, a cellulose ester 20 which is readily soluble therein, in proportions to form a solution containing not less than 29% of said ester, and adding thereto suitable proportions of an oil and a filling material.
- 25 7. In the manufacture of a celluloid substitute, the process which comprises dissolving, in a mixture comprising alcohol and a chlorinated hydrocarbon, a cellulose ester which is readily soluble therein, and in adding thereto suitable proportions of an oil, a filling material and a coloring material.
8. In a process of making a celluloid substitute, the step which comprises dissolving in a mixture comprising alcohol and a plurality of chlorinated hydrocarbons, a cellulose ester which is readily soluble therein, in proportions to form a solution containing not less than 29% of said ester.
9. In a process of making a celluloid substitute, the step which comprises dissolving 40 in a mixture comprising alcohol and tetrachlorethane and another chlorinated hydrocarbon, a cellulose ester which is readily soluble therein, in proportions to form a solution containing not less than 29% of said ester.
- 45 10. In a process of making a celluloid substitute, the step which comprises dissolving in a mixture comprising alcohol and a cellulose ester which is readily soluble therein, in proportions to form a solution containing about 50% of said ester.
11. A process of making a celluloid substitute, which comprises dissolving in a mixture comprising alcohol, tetrachlorethane, and pentachlorethane, a cellulose ester which is readily soluble therein, in proportions to form a solution containing not less than 29% of said ester.
12. A celluloid substitute having a cellulose ester readily soluble in a mixture of alcohol and tetrachlorethane as a base, said product being relatively noninflammable, nonbrittle, transparent, and capable of being worked up in the same manner as celluloid.
13. A celluloid substitute having cellulose acetate soluble in a mixture of alcohol and tetrachlorethane as a base, containing an oil, said product being relatively noninflammable, nonbrittle, transparent, and capable of being worked up in the same manner as celluloid.
14. A celluloid substitute having cellulose acetate soluble in a mixture of alcohol and tetrachlorethane as a base, containing coloring material and an oil, said product being relatively noninflammable, nonbrittle, transparent, and capable of being worked up in the same manner as celluloid.
- In testimony whereof I have hereunto set my hand in the presence of two subscribing witnesses.
- Paris, dated this 20th day of September 1911.
- DR. HENRY DREYFUS.
- Witnesses:
- H. C. COXE,  
CAMILLE DREYFUS.